# EUROPEAN PATENT SPECIFICATION

(11) **EP 2 065 478 B1**
(45) Date of publication and mention of the grant of the patent: **13.02.2019**
(21) Application number: 08170293.8
(22) Date of filing: 28.11.2008
(51) Int. Cl.: C22C 1/00, C22C 16/00, C22C 45/10

(54) **A ZR-BASED AMORPHOUS ALLOY AND A PREPARATION METHOD THEREOF**
ZR-BASIERTE AMORPHE LEGIERUNG UND HERSTELLUNGSVERFAHREN DAFÜR
ALLIAGE AMORPHE À BASE DE ZR ET SON PROCÉDÉ DE PRÉPARATION

(30) Priority: 30.11.2007 CN 200710187786
(43) Date of publication of application: 03.06.2009
(73) Proprietor: Byd Company Limited, Shenzhen 518118 (CN)
(72) Inventor: Lu, Kun, Shenzhen 518118 (CN); Jiang, Linlin, Shenzhen 518118 (CN); Zhang, Faliang, Shenzhen 518118 (CN); Gong, Qing, Shenzhen 518118 (CN)
(74) Representative: Epping - Hermann - Fischer

(56) References cited:
- ZHAO, DEQIAN; WANG, WEIHUA; ZHUANG, YANXIN; PAN MINGXIANG; JI, YINGFEI; MA, XUEMING: "FORMATION AND PERFORMANCE OF NEW ZR-TI-CU-NI-BE-FE BULD AMORPHOUS ALLOY" SCIENCE IN CHINA (SERIES A), [Online] vol. 43, no. 3, 1 March 2000 (2000-03-01), pages 307-311, XP002512309 ISSN: 1862-2763 Retrieved from the Internet: URL:http://www.springerlink.com/content/62 188vn764568505/> [retrieved on 2009-01-27]
- SUN,JIAN-FEI;SHEN,JUN;GAO,YUI-LAI: "Effect of Sn addition on thermal stability of (Zr52.5Ti5Al10Ni14.6Cu17.9)(100-x)Snx alloys" TRANS. NONFERROUS MET. SOC. CHINA, vol. 13, May 2003 (2003-05), pages 64-67, XP008101301
- JOHNSON W L: "Fundamental aspects of bulk metallic glass formation in multicomponent alloy" MATERIALS SCIENCE FORUM, AEDERMANNSFDORF, CH, vol. 225-227, 1 January 1996 (1996-01-01), pages 35-50, XP008100967 ISSN: 0255-5476

## Description

### FIELD OF THE DISCLOSURE

The present disclosure relates to a Zr-based amorphous alloy and a preparing method thereof.

### BACKGROUND OF THE DISCLOSURE

Amorphous metallic alloys are disordered in the long range but ordered in the short range. They have desirable physical and chemical properties, such as high strength, high hardness, high wearing resistance, high corrosion resistance, relatively wide elastic range, high electric resistance, good superconductivity, and low magnetic loss. Amorphous metallic alloys have huge potential when used as structural materials. They are widely used in many fields such as mechanics, IT electronics, the military industry and so on.

However, some characteristics of the amorphous metallic alloys limit their applications. For example, it is difficult to manufacture large size amorphous alloys. To obtain the disordered structure in the long range, atoms' spontaneous movement in the freezing process shall be restrained. The higher the cooling speed is, the lower the possibility is for the atoms to form orderly arrayed crystalline materials via spontaneous movement. But as product size increases, the internal cooling speed within the product is declining. Thus, the internal amorphous degree is low in the long range and it is difficult to form large size amorphous structures.

Also, it is difficult to effectively improve the plasticity characteristics of the amorphous materials. Due to their particular structure, while under stress, the amorphous alloy materials do not have the internal deformation mechanism as crystalline materials do in order to resist deformation. So when the stress reaches a certain degree, the amorphous alloy material may break suddenly, which may lead to catastrophic accidents. Thus, the applications of the amorphous alloy materials as structural materials are limited.

Zhao et al. discloses a Zr-Ti-Cu-Ni-Be-Fe bulk amorphous alloy and its preparing method (Forming And Performance of The Zr-Ti-Cu-Ni-Be-Fe Bulk Amorphous Alloy And Amorphous-Based Nano-Composite, Zhao De Qian, Zhang Yong, Pan Ming Xiang, Meng Li Qin, Wang Wei Hua, Acta Metallurgica Sinica, March, 2000). The method comprises adding 2-10 atomic percent of Fe to form a nano crystalline composite material in order to change the magnetic susceptibility of the material. As a result of the addition of Fe in increasing amount, sharp diffraction peaks begin to appear in the XRD diagram, indicating crystallization. It shows that the addition of relatively large amount of iron is effective in affecting the amorphous alloy forming ability. Zhao et al. however does not address the issues of large size amorphous alloy manufacturing and the plasticity of the amorphous alloy materials. Zhao et al. "Formation and Performance of New Zr-Ti-Cu-Ni-Be-Fe Bulk Amorphous Alloy" Science in China (series A) vol. 43, no. 3, pages 307 to 311 reports the formation of the new Zr-Ti-Cu-Ni-Be-Fe bulk amorphous alloy with high strength.

### SUMMARY OF THE DISCLOSURE

The present invention provides a Zr-based amorphous alloy according to claim 1 and a method for the preparation thereof according to claim 6. Preferred embodiments are set forth in the subclaims.

### DESCRIPTION OF THE DRAWINGS

Fig. 1 is the quasi-three component phase diagram (Zr, Ti, Sn)-(Cu, Ni)-(Be, Fe) of the amorphous alloy.
Fig. 2 is the stress-strain diagram of the amorphous alloy prepared in Example 1 and Control 1.
Fig. 3 is the XRD diagram of the amorphous alloy prepared in the Examples 1-5 and Control 1.

### DETAILED DESCRIPTION OF THE PREFERRED EMBODIMENTS

According to one embodiment of the present disclosure, a Zr-based amorphous alloy as defined in claim 1 is provided. Preferred embodiments are set forth in the subclaims.

Referring to Fig. 1, the quasi-three component phase diagram of the amorphous alloy composition is shown. The large parallelogram area is the amorphous alloy forming area, the boundary of which is determined by the composition range of the amorphous alloy according to one embodiment of the present disclosure. The small parallelogram area is the preferred amorphous alloy forming area, the boundary of which is determined by the preferred composition range of the amorphous alloy according to one embodiment of the present disclosure. The three vertexes of the quasi-three component phase diagram respectively represent the elements in the amorphous alloy. The alloy in Fig. 1 does not include ETM and LTM. The numbers on each axis represent the atomic percentages of the elements in the alloy.

According to another embodiment of the present disclosure, a method for preparing a Zr-based amorphous alloy as defined in claim 6 is provided. The method comprises vacuum melting an amorphous alloy material and cooling the amorphous alloy material to form an amorphous alloy, both under inert gas.

The material for preparing the Zr-based amorphous alloy comprises Zr, Ti, Cu, Ni, Fe, and Be. The material for preparing the Zr-based amorphous alloy also comprises Sn, and optionally ETM and LTM.

The amount of each element added should be adjusted such that the elements in the raw material have the following formula: (ZrₓTi_{y}Sn_{z})ₐ : ETM_{b} : (CuₘNiₙ)_{c} : Fe_{d} : LTMₑ : Be_{f}, wherein a, b, c, d, e and f, x, y and z, m and n, ETM, and LTM are as defined above.

In a preparing method for a Zr-based amorphous alloy, any suitable melting method can be used. For example, the melted raw materials should be mixed first, and then cooled to form ingots. In this step, the raw materials can be melted in an electric arc melting equipment or an induction melting equipment. The melting temperature and time differ to some extent according to the heating process selected. Usually, the melting temperature can be about 1000-2700°C, preferably about 1500-2000°C. The melting time is about 5-20 minutes. The vacuum level is not higher than about 200 Pa, preferably about 0.01-5 Pa.

As a pre-process before molding, the ingots were crushed as if the molding process need. The ingots then can be re-melted and molding.. Electric arc melting, induction melting, and resistance melting are commonly used in the re-melting process. The re-melting temperature can be about 1000-2300°C, preferably about 1000-1500°C. The vacuum level is not higher than about 200 Pa, preferably about 0.01-5 Pa. Any suitable molding method can be used to form the amorphous alloy. For example, melt-spinning, copper mold casting, suction casting, die casting, jetting molding, or water quenching can be used. The cooling speed of the molding process can be about 10-10⁴ K/s. Since the critical dimensions differ among different components, different molding methods can be selected. The inert gas can be one or more elements selected from the SF₆ gas and Group Zero elements of the Element Periodic Table.

### Example 1

A preparation method of a Zr-based amorphous alloy is illustrated in this example.

Raw materials Zr, Ti, Sn, Cu, Ni, Fe, Be (about 25 grams) were added to an electric arc melting equipment (Shen Yang Scientific Instrument Manufacturing Company Limited). The formulars of the raw materials were as follows: (Zr_{0.74}Ti_{0.25}Sn_{0.01})_{55.34}(Cu_{0.56}Ni_{0.44})_{20.65}Fe_{1.96}Be_{22.05}. The equipment was vacuumized to about 5 Pa. The raw material was melted at about 2000 °C under Ar protection for about 6 minutes. The molten master alloy was mixed sufficiently, and then cooled into an ingot. The ingot was re-melted at about 1500 °C using electric arc melting, and then cooled in a copper mold casting process with a cooling speed of about 10² k/s to obtain the Zr-based amorphous alloy sample C1.

### Example 2

Another preparation method of a Zr-based amorphous alloy is illustrated in this example.

Raw materials Zr, Ti, Sn, Cu, Ni, Fe, Be (about 200 kg) were added to an induction melting equipment (Zhongbei Technology). The formulars of the raw materials were as follows: (Zr_{0.74}Ti_{0.25}Sn_{0.01})_{55.34}(Cu_{0.56}Ni_{0.44})_{20.65}Fe_{1.96}Be_{22.05}. The equipment was vacuumized to about 5 Pa. The raw materials were melted at about 1800 °C under Ar protection for about 10 minutes. The molten master alloy was mixed sufficiently, and then cooled into an ingot. The ingot was re-melted at about 1200 °C using resistance heating, and then cooled in a die-casting process with a cooling speed of about 10⁴ k/s to obtain the Zr-based amorphous alloy sample C2.

### Example 3

Yet another preparation method of a Zr-based amorphous alloy is illustrated in this example.

Raw materials Zr, Ti, Sn, Cu, Ni, Fe, Be (about 20 g) were added to a quartz tube (Zhongbei Technology). The formulars of the raw materials were as follows: (Zr_{0.80}Ti_{0.17}Sn_{0.03})₄₀Y₅Nb₅(Cu_{0.64}Ni_{0.36})₂₅Fe₅Be₂₀. The tube was vacuumized to about 200 Pa. The raw materials were melted at about 2000 °C by induction heating under Ar protection for about 5 minutes. The molten master alloy was mixed sufficiently, and then cooled into an ingot. The ingot was re-melted at about 1500 °C by induction heating, and then cooled in a water quenching process with a cooling speed of about 10³ k/s to obtain the Zr-based amorphous alloy sample C3.

### Example 4

Still another preparation method of a Zr-based amorphous alloy is illustrated in this example.

Raw materials Zr, Ti, Sn, Cu, Ni, Fe, Be (about 200 kg) were added into an induction melting equipment. The formulas of the raw materials were as follows: (Zr_{0.65}Ti_{0.29}Sn_{0.06})₅₀(Cu_{0.5}Ni_{0.5})₂₀Co₁₀Fe₃Be₁₇. The equipment was vacuumized to about 5 Pa. The raw materials were induction melted at about 1800 °C under Ar protection for about 10 minutes. The molten master alloy was mixed sufficiently, and then cooled it into an ingot. The ingot was re-melted at about 1000 °C by resistance heating, and then was melt-spinned with a cooling speed of about 10⁴ k/s to obtain the Zr-based amorphous alloy sample C4.

### Example 5

Yet still another preparation method of a Zr-based amorphous alloy is illustrated in this example.

Raw materials Zr, Ti, Sn, Cu, Ni, Fe, Be (about 20 g) were added into a quartz tube (Middle North Technology). The formulas of the raw materials were as follows: (Zr_{0.75}Ti_{0.24}Sn_{0.01})₆₀W₃(Cu_{0.55}Ni_{0.45})₁₅Pd₂Zn₁Fe₄Be₁₅. The tube was vacuumized to about 2×10⁻² Pa. The raw materials were induction melted at about 2000 °C under Ar protection for about 5 minutes. The molten master alloy was mixed sufficiently, and then cooled into an ingot. The ingot was re-melted at about 1500 °C by induction heating, and then cooled in a water quenching process with a cooling speed of about 10⁴ k/s to obtain the Zr-based amorphous alloy sample C5.

### Control 1

The control illustrates an amorphous material prepared according to the present art.

Raw materials Zr, Ti, Cu, Ni, Be, Fe (about 25 grams) were added into an electric arc melting equipment (Shen Yang Technical Instruments Manufacture Company Limited). The formulas of the raw materials were as follows: Zr₄₁Ti₁₄Cu₁₁Ni_{9.5}Fe₂Be_{22.5}. The equipment was vacuumized to about 5 Pa. The starting materials were melted at about 2000 °C under Ar protection for about 6 minutes. The molten master alloy was mixed sufficiently, and then cooled into an ingot. The ingot was re-melted at about 1500 °C by electric arc melting, and then was copper mold cast with a cooling speed of about 10² k/s to obtain the Zr-based amorphous alloy sample D1.

### Experimental:

### Testing methods

### (1) Compression test

The samples were tested on a XinSansi CMT5000 series testing machine with a measuring range of 30KN and a loading speed of about 0.5 mm/minute. The stress-strain conditions of the sample C1 and D1 were tested. The test results are showed in Fig 2.

### (2) Hardness test

The samples were tested on a Micro Hardness Text Hv1000 Vickers Hardness Testing Machine. The weight of the pressure head was about 200 g, and the loading time was about 10 seconds. Datas of three test points were obtained for each sample to calculate the arithmetic average value. The results are showed in Table 1.

### (3) XRD analysis

XRD analyzes the physical phase of an alloy material in order to estimate whether the alloy is amorphous. The samples were made into powder for test on a Model D-MAX2200PC X-ray Powder Diffractometer. Using a Cu Kα radiation. The incidence wave length λ was about 1.54060 Å. The accelerating voltage was about 40 kV. The current was about 20 mA. Step scan was used with a step size of about 0.04 degree. The test results are showed in Fig 3.

### (4) The test of critical dimensions

A wedged sample formed in the copper mold casting process was cut from the top by a thickness of about 1 mm. The cross section after cutting was analyzed by XRD. The structure type was determined. If the structure type was an amorphous alloy, then the cutting process was continued until the structure was no longer an amorphous alloy. The total cutting thickness was recorded. The critical dimension was the total cutting thickness minus 1 mm. The results are showed in Table 1.

**Table 1**

| Serial No. | C1 | C2 | C3 | C4 | C5 | D1 |
|---|---|---|---|---|---|---|
| Critical Dimension (mm) | >14 | >14 | 14 | 12 | 12 | 8 |
| Average Hardness (Hv) | 553 | 553 | 547 | 539 | 548 | 537 |

From the results showed in Table 1, the Zr-based amorphous alloys provided according to embodiments of the present disclosure have critical dimensions larger than about 1 centimeter. Meanwhile, they have relatively higher hardness. As shown in Fig. 3, there are no sharp diffraction peaks in the XRD diagrams of Sample C1, C2, C3, C4, C5 and D1, which indicates the alloys have a high degree of amorphization. As shown in Fig. 2, the Zr-based amorphous alloy C1 provided according to one embodiment of the present disclosure and the Zr-based amorphous alloy D1 provided according to the prior art assume substantially overlapping curves in the low stress area when identical stresses were applied. However, as the stresses increased, D1 could only sustain a relatively low strain, and would break easily. Meanwhile, the curve representing the C1 alloy was bending, which indicates that the strain capacity of the C1 alloy is much better than D1, that is, the Zr-based amorphous alloy according to embodiments of the present disclosure has better plasticity.

## Claims

1. A Zr-based amorphous alloy, consisting of
40-75 atomic percent of (ZrₓTi_{y}Sn_{z}),
10-35 atomic percent of (CuₘNiₙ),
0.5-5 atomic percent of Fe,
15-25 atomic percent of Be,
0-10 atomic percent of ETM, and
0-10 atomic percent of LTM,
wherein x, y and z are atomic fractions, and x+y+z equals to 1;
wherein x is 0.6-0.85, and z is in the range of 0.01x - 0.1x;
wherein m and n are atomic fractions, and m+n equals to 1; and
wherein m is 0.5-0.65
wherein ETM comprises at least one element selected from Group IIIB, Group IVB, Group VB and Group VIB of the Element Periodic Table, provided that ETM is not Zr or Ti, and
wherein LTM comprises at least one element selected from Group IB, Group IIB, Group VIIB, Group VIIIB of the Element Periodic Table, provided that LTM is not Cu, Ni or Fe.

2. The amorphous alloy according to claim 1, wherein ETM is one or two elements selected from the Group consisting of Sc, Y, La, Ce, Pr, Nd, Hf, V, Nb, Ta, Cr, Mo, and W, and wherein LTM is one or two elements selected from the Group consisting of Mn, Tc, Re, Ru, Os, Co, Rh, Ir, Pd, Pt, Ag, Au, Zn, Cd, and Hg, preferably ETM and LTM together comprises 1-3 elements.

3. The amorphous alloy according to claim 1 or 2, which consists of 40-60 atomic percent of (ZrₓTi_{y}Sn_{z}), and 15-25 atomic percent of (CuₘNiₙ).

4. The amorphous alloy according to any one of claims 1 to 3, the critical dimension of which is large than 1cm.

5. The Zr-based amorphous alloy of claim 1, wherein said alloy consists of 40-75 atomic percent of (ZrₓTi_{y}Sn_{z}), 10-35 atomic percent of (CuₘNiₙ), 0.5-5 atomic percent of Fe, and 15-25 atomic percent of Be,
wherein x, y and z are atomic fractions, and x+y+z equals to 1,
wherein x is 0.6-0.85, and z is in the range of 0.01x - 0.1x;
wherein m and n are atomic fractions, and m+n equals to 1; and
wherein m is 0.5-0.65.

6. A method for preparing a Zr-based amorphous alloy according to any one of claims 1 to 5: melting a raw material comprising Zr, Ti, Cu, Ni, Fe, Be, and Sn under a vacuum of less than 200 Pa to form an alloy mixture under a vacuum circumstance; and molding the alloy mixture and cooling to form the amorphous alloy wherein the cooling speed of the cooling molding process is 10-10⁴ K/s.

7. The method according to claim 6, wherein the raw material further comprises one or both of ETM and LTM, wherein ETM comprises at least one element selected from Group IIIB, Group IVB, Group VB and Group VIB of the Element Periodic Table, provided that ETM is not Zr or Ti, preferably ETM is one or two elements selected from the Group consisting of Sc, Y, La, Ce, Pr, Nd, Hf, V, Nb, Ta, Cr, Mo, and W, wherein LTM comprises at least one element selected from Group IB, Group IIB, Group VIIB, Group VIIIB of the Element Periodic Table, provided that LTM is not Cu, Ni or Fe, preferably LTM is one or two elements selected from the Group consisting of Mn, Tc, Re, Ru, Os, Co, Rh, Ir, Pd, Pt, Ag, Au, Zn, Cd, and Hg, more preferably ETM and LTM together comprises 1-3 elements.

8. The method according to claim 6 or 7, wherein the elements in the raw material have the following formula:
Zr_{g} : Tiₕ : Snᵢ : ETM_{b} : (Cuₖ : Niₗ : Fe_{d} : LTMₑ : Be_{f},
wherein b, d, e, f, g, h, i, k and 1 are atomic percentages;
wherein g is 24-63.75 %, preferably 24-51 %, h is 2.6-29.55 %, preferably , 2.6-23.64, i is 0.24-6.375 %, preferably 0.24 - 5.1 %, b is 0-10%, k is 5-22.75%, preferably 7.5-16.25%, 1 is 3.5-17.5%, preferably 5.25-12.5%, d is 0.5-5%, e is 0-10%, and f is 15-25%,
with the proviso that the amount of Zr, Ti and Sn adds up to 40-75 atomic percent, the proviso that the atomic amount of Sn is 1% - 10 of the atomic amount of Zr, the proviso that the amount of Cu and Ni adds up to 10-35 atomic percent, preferably 15-25 atomic percent and the proviso that the atomic amount of Ni is 53.85% - 100% of the atomic amount of Cu.

9. The method according to any one of claims 6 to 8, wherein the melting step comprises:
melting the raw material to form a molten mixture;
cooling the molten mixture to form at least one ingot; and
re-melting the at least one ingot to form the alloy mixture.

10. The method according to any one of claims 6 to 9, wherein the raw material is melted under a vacuum of less than 5 Pa.

11. The method according to any one claims 6 to 10, wherein the raw material is melted at a temperature of 1000 - 2700 °C.

12. The method according to any one of claims 6 to 11, wherein the molding is a cold molding process.

13. The method according to any one of claims 6 to 12, wherein the molding is a process selected from a Group consisting of melt-spinning, copper mold casting, suction casting, die casting, jetting molding, and water quenching.

14. The method according to any one of claims 6 to 13, wherein the raw material is melted in the presence of an inert gas, preferably in the presence of one or more gases selected from the Group consisting of SF₆ and Group Zero gases.

## Patentansprüche

1. Zr-basierte amorphe Legierung, bestehend aus:
40-75 Atomprozent (ZrₓTi_{y}Sn_{z})
10-35 Atomprozent (CuₘNiₙ),
0,5-5 Atomprozent Fe,
15-25 Atomprozent Be,
0-10 Atomprozent eines frühen Übergangsmetalls (ETM), und
0-10 Atomprozent eines späten Übergangsmetalls (LTM),
wobei es sich bei x, y und z um Atombrüche handelt und x+y+z gleich 1 ist;
wobei x 0,6-0,85 beträgt, und z in dem Bereich von 0,01x bis 0,1x liegt;
wobei es sich bei m und n um Atombrüche handelt und m+n gleich 1 ist; und
wobei m 0,5-0,65 beträgt
wobei das ETM zumindest ein Element ausgewählt aus der Gruppe IIIB, Gruppe IVB, Gruppe VB und Gruppe VIB des Periodensystems der Elemente aufweist, vorausgesetzt bei dem ETM handelt es sich nicht um Zr oder Ti, und
wobei das LTM zumindest ein Element ausgewählt aus der Gruppe IB, Gruppe IIB, Gruppe VIIB, Gruppe VIIIB des Periodensystems der Elemente aufweist, vorausgesetzt bei dem LTM handelt es sich nicht um Cu, Ni oder Fe.

2. Amorphe Legierung nach Anspruch 1, wobei es sich bei dem ETM um ein oder zwei Element(e) ausgewählt aus der Gruppe bestehend aus Sc, Y, La, Ce, Pr, Nd, Hf, V, Nb, Ta, Cr, Mo und W handelt, und wobei es sich bei dem LTM um ein oder zwei Element(e) ausgewählt aus der Gruppe bestehend aus Mn, Tc, Re, Ru, Os, Co, Rh, Ir, Pd, Pt, Ag, Au, Zn, Cd und Hg handelt, vorzugsweise umfassen das ETM und das LTM zusammen 1-3 Elemente.

3. Amorphe Legierung nach Anspruch 1 oder 2, die aus 40-60 Atomprozent (ZrₓTi_{y}Sn_{z}) und 15-25 Atomprozent (CuₘNiₙ) besteht.

4. Amorphe Legierung nach einem der Ansprüche 1 bis 3, deren kritische Größe mehr als 1 cm beträgt.

5. Zr-basierte amorphe Legierung nach Anspruch 1, wobei besagte Legierung aus 40-75 Atomprozent (ZrₓTi_{y}Sn_{z}), 10-35 Atomprozent (CuₘNiₙ), 0,5-5 Atomprozent Fe und 15-25 Atomprozent Be besteht,
wobei es sich bei x, y und z um Atombrüche handelt und x+y+z gleich 1 ist,
wobei x 0,6-0,85 beträgt, und z in dem Bereich von 0,01x bis 0,1x liegt;
wobei es sich bei m und n um Atombrüche handelt und m+n gleich 1 ist; und
wobei m 0,5-0,65 beträgt.

6. Verfahren zur Herstellung einer Zr-basierten amorphen Legierung nach einem der Ansprüche 1 bis 5: Schmelzen eines Rohstoffs umfassend Zr, Ti, Cu, Ni, Fe, Be und Sn in einem Vakuum von weniger als 200 Pa zur Bildung eines Legierungsgemisches unter einer Vakuumbedingung; und Formung des Legierungsgemisches und Kühlung zur Bildung der amorphen Legierung, wobei die Abkühlgeschwindigkeit des Formkühlungsprozesses 10-10⁴ K/s beträgt.

7. Verfahren nach Anspruch 6, wobei der Rohstoff außerdem eines oder beide von dem ETM und dem LTM umfasst, wobei das ETM zumindest ein Element ausgewählt aus Gruppe IIIB, Gruppe IVB, Gruppe VB und Gruppe VIB des Periodensystems der Elemente aufweist, vorausgesetzt bei dem ETM handelt es sich nicht um Zr oder Ti, vorzugsweise es sich bei dem ETM um ein oder zwei Element(e) ausgewählt aus der Gruppe bestehend aus Sc, Y, La, Ce, Pr, Nd, Hf, V, Nb, Ta, Cr, Mo und W handelt, wobei das LTM zumindest ein Element ausgewählt aus der Gruppe IB, Gruppe IIB, Gruppe VIIB, Gruppe VIIIB des Periodensystems der Elemente aufweist, vorausgesetzt bei dem LTM handelt es sich nicht um Cu, Ni oder Fe, vorzugsweise es sich bei dem LTM um ein oder zwei Element(e) ausgewählt aus der Gruppe bestehend aus Mn, Tc, Re, Ru, Os, Co, Rh, Ir, Pd, Pt, Ag, Au, Zn, Cd und Hg handelt, ferner bevorzugt das ETM und das LTM zusammen 1-3 Elemente aufweisen.

8. Verfahren nach Anspruch 6 oder 7, wobei die Elemente in dem Rohstoff die folgende Formel haben:
Zr_{g} : Tiₕ : Snᵢ: ETM_{b} : (Cuₖ : Niₗ: Fe_{d} : LTMₑ : Be_{f},
wobei es sich bei b, d, e, f, g, h, i, k und l um Atomprozente handelt;
wobei g 24-63,75 % beträgt, vorzugsweise 24-51 %, h 2,6-29,55 % beträgt, vorzugsweise 2,6-23,64, i 0,24-6,375 % beträgt, vorzugsweise 0,24-5,1 %, b 0-10 % beträgt, k 5-22,75 % beträgt, vorzugsweise 7,5-16,25 %, 13,5-17,5 % beträgt, vorzugsweise 5,25-12,5 %, d 0,5-5 % beträgt, e 0-10 % beträgt und f 15-25 % beträgt,
mit der Maßgabe, dass die Menge von Zr, Ti und Sn 40-75 Atomprozent beträgt, der Maßgabe, dass die Atommenge von Sn 1 % - 10 der Atommenge von Zr beträgt, der Maßgabe, dass die Menge von Cu und Ni 10-35 Atomprozent ergibt, vorzugsweise 15-25 Atomprozent, und der Maßgabe, dass die Atommenge von Ni 53,85 % - 100 % der Atommenge von Cu beträgt.

9. Verfahren nach einem der Ansprüche 6 bis 8, wobei der Schmelzschritt umfasst:
Schmelzen des Rohstoffs zur Bildung eines Schmelzegemisches;
Kühlung des Schmelzegemisches zur Bildung zumindest eines Blocks; und
Umschmelzen des zumindest einen Blocks zur Bildung der Legierungsmischung.

10. Verfahren nach einem der Ansprüche 6 bis 9, wobei der Rohstoff in einem Vakuum von weniger als 5 Pa geschmolzen wird.

11. Verfahren nach einem der Ansprüche 6 bis 10, wobei der Rohstoff bei einer Temperatur von 1.000 - 2.700 °C geschmolzen wird.

12. Verfahren nach einem der Ansprüche 6 bis 11, wobei es sich bei der Formung um ein Kaltumformungsverfahren handelt.

13. Verfahren nach einem der Ansprüche 6 bis 12, wobei es sich bei der Formung um einen Prozess ausgewählt aus einer Gruppe bestehend aus Rascherstarrung, Kupferformgießen, Sauggießen, Druckgießen, Spritzgießen und Wasserquenchen handelt.

14. Verfahren nach einem der Ansprüche 6 bis 13, wobei der Rohstoff in Gegenwart von einem Inertgas geschmolzen wird, vorzugsweise in Gegenwart von einem oder mehreren Gas(en) gewählt aus der Gruppe bestehend aus SF₆ und Gasen der Gruppe Null.

## Revendications

1. Alliage amorphe à base de Zr, consistant en :
40-75 en pourcentage atomique de (ZrₓTi_{y}Sn_{z}) ;
10-35 en pourcentage atomique de (CuₘNiₙ) ;
0,5-5 en pourcentage atomique de Fe ;
15-25 en pourcentage atomique de Be ;
0-10 en pourcentage atomique d'ETM, et
0-10 en pourcentage atomique de LTM ;
dans lequel x, y, et z sont des fractions atomiques, et x+y+z équivaut à 1 ;
dans lequel x est 0,6-0,85, et z est compris dans la plage de 0,01x - 0,1x ;
dans lequel m et n sont des fractions atomiques, et m+n équivaut à 1, et
dans lequel m est 0,5-0,65 ;
dans lequel ETM comprend au moins un élément sélectionné parmi le groupe IIIB, le groupe IVB, le groupe VB, et le groupe VIB du tableau périodique des éléments, à condition que ETM ne soit pas Zr ou Ti, et
dans lequel LTM comprend au moins un élément sélectionné parmi le groupe IB, le groupe IIB, le groupe VIIB, et le groupe VIIIB du tableau périodique des éléments, à condition que LTM ne soit pas Cu, Ni ou Fe.

2. Alliage amorphe selon la revendication 1, dans lequel ETM est un ou deux éléments sélectionnés parmi le groupe consistant en Sc, Y, La, Ce, Pr, Nd, Hf, V, Nb, Ta, Cr, Mo et W, et dans lequel LTM est un ou deux éléments sélectionnés parmi le groupe consistant en Mn, Tc, Re, Ru, Os, Co, Rh, Ir, Pd, Pt, Ag, Au, Zn, Cd et Hg, et de préférence ETM et LTM ensemble comprennent de 1 à 3 éléments.

3. Alliage amorphe selon la revendication 1 ou 2, lequel consiste en 40-60 en pourcentage atomique de (ZrₓTi_{y}Sn_{z}), et en 15-25 en pourcentage atomique de (CuₘNiₙ).

4. Alliage amorphe selon l'une quelconque des revendications 1 à 3, dont la dimension critique est supérieure à 1 cm.

5. Alliage amorphe selon la revendication 1, dans lequel ledit alliage consiste en 40-75 en pourcentage atomique de (ZrₓTi_{y}Sn_{z}), 10-35 en pourcentage atomique de (CuₘNiₙ), 0,5-5 en pourcentage atomique de Fe, et 15-25 en pourcentage atomique de Be ;
dans lequel x, y, et z sont des fractions atomiques, et x+y+z équivaut à 1 ;
dans lequel x est 0,6-0,85, et z est compris dans la plage de 0,01x - 0,1x ;
dans lequel m et n sont des fractions atomiques, et m+n équivaut à 1, et
dans lequel m est 0,5-0,65.

6. Procédé destiné à préparer un alliage amorphe à base de Zr selon l'une quelconque des revendications 1 à 5, comprenant l'étape pour faire fondre une matière première comprenant du Zr, Ti, Cu, Ni, Fe, Be et Sn sous un vide inférieur à 200 Pa afin de former un mélange d'alliage sous une condition de vide, et pour mouler le mélange d'alliage et refroidir afin de former l'alliage amorphe, dans lequel la vitesse de refroidissement du processus de moulage et refroidissement est de 10-10⁴ K/s.

7. Procédé selon la revendication 6, dans lequel la matière première comprend en outre un élément parmi ETM et LTM, ou les deux ; dans lequel ETM comprend au moins un élément sélectionné parmi le groupe IIIB, le groupe IVB, le groupe VB, et le groupe VIB du tableau périodique des éléments, à condition que ETM ne soit pas Zr ou Ti ; de préférence ETM est un ou deux éléments sélectionnés parmi le groupe consistant en Sc, Y, La, Ce, Pr, Nd, Hf, V, Nb, Ta, Cr, Mo et W, et dans lequel LTM comprend au moins un élément sélectionné parmi le groupe IB, le groupe IIB, le groupe VIIB, et le groupe VIIIB du tableau périodique des éléments, à condition que LTM ne soit pas Cu, Ni ou Fe ; de préférence, LTM est un ou deux éléments sélectionnés parmi le groupe consistant en Mn, Tc, Re, Ru, Os, Co, Rh, Ir, Pd, Pt, Ag, Au, Zn, Cd et Hg, et de préférence ETM et LTM comprennent ensemble de 1 à 3 éléments.

8. Procédé selon la revendication 6 ou 7, dans lequel les éléments dans la matière première présentent la formule suivante :
Zr_{g} : Tiₕ : Snᵢ : ETM_{b} : (Cuₖ : Niₗ : Fe_{d} : LTMₑ : Be_{f} ;
dans lequel b, d, e, f, g, h, i, k et l sont des pourcentages atomiques ;
dans lequel g est 24-63,75 %, et de préférence 24-51 % ; h est 2,6-29,55 %, et de préférence 2,6-23,64 % ; i est 0,24-6,375 %, et de préférence 0,24-5,1 % ; b est 0-10 % ; k est 5-22,75 %, et de préférence 7,5-16,25 % ; l est 3,5-17,5 %, et de préférence 5,25-12,5 % ; d est 0,5-5 % ; e est 0-10 %, et f est 15-25 % ;
à condition que la quantité de Zr, Ti et Sn soit additionnée de manière à atteindre 40-75 en pourcentage atomique ; à condition que la quantité atomique de Sn soit 1 %-10 de la quantité atomique de Zr ; à condition que la quantité de Cu et Ni soit additionnée de manière à atteindre 10-35 en pourcentage atomique, et de préférence 15-25 en pourcentage atomique, et à condition que la quantité atomique de Ni soit 53,85 %-100 % de la quantité atomique de Cu.

9. Procédé selon l'une quelconque des revendications 6 à 8, dans lequel l'étape de fusion comprend les étapes de :
faire fondre la matière première afin de former un mélange fondu ;
refroidir le mélange fondu afin de former au moins un lingot, et
faire fondre à nouveau le au moins un lingot afin de former le mélange d'alliage.

10. Procédé selon l'une quelconque des revendications 6 à 9, dans lequel la matière première est fondue sous un vide inférieur à 5 Pa.

11. Procédé selon l'une quelconque des revendications 6 à 10, dans lequel la matière première est fondue à une température de 1000 à 2700 °C.

12. Procédé selon l'une quelconque des revendications 6 à 11, dans lequel le moulage est un processus de moulage à froid.

13. Procédé selon l'une quelconque des revendications 6 à 12, dans lequel le moulage est un processus sélectionné parmi un groupe consistant en un filage à l'état fondu, une coulée en moules de cuivre, une coulée sous vide, une coulée sous pression, un moulage par jet, et une trempe à l'eau.

14. Procédé selon l'une quelconque des revendications 6 à 13, dans lequel la matière première est fondue en présence d'un gaz inerte, de préférence en présence d'un ou de plusieurs gaz sélectionnés parmi le groupe consistant en SF₆ et le groupe des gaz à pression zéro.
